

F. BLAU.

MANUFACTURE OF FINE REFRACTORY METAL WIRES.

APPLICATION FILED JAN. 31, 1912.

1,157,288.

Patented Oct. 19, 1915.



Witnesses:

Helen Orford

Margaret E. Shoolley

Inventor:  
Fritz Blau,  
by Alberts, Davis  
His Attorney.

# UNITED STATES PATENT OFFICE.

FRITZ BLAU, OF CHARLOTTENBURG, GERMANY, ASSIGNOR TO GENERAL ELECTRIC COMPANY, A CORPORATION OF NEW YORK.

## MANUFACTURE OF FINE REFRACtORY-METAL WIRES.

1,157,288.

Specification of Letters Patent. Patented Oct. 19, 1915.

Application filed January 31, 1912. Serial No. 674,476.

To all whom it may concern:

Be it known that I, Dr. FRITZ BLAU, a subject of the Emperor of Austria-Hungary, residing at Charlottenburg, Germany, have invented certain new and useful Improvements in the Manufacture of Fine Refractory-Metal Wires, of which the following is a specification.

My invention relates to refractory metal wire and ribbon and to its production.

By my process of manufacture tungsten filaments or wires can be produced of a fineness and uniformity greatly superior to anything heretofore made or obtainable in any way, and this wire is of remarkable uniformity of section for any length desired and of perfectly uniform surface; indeed, extremely small diameters for which the well known Wollaston process entirely fails can readily be obtained in any desired lengths. Moreover, the process is easily carried out, and even when the wire is not reduced below what has hitherto been the extreme limit of fineness, the production of tungsten wire (especially of the finer sizes) is rendered very much easier and cheaper.

Other advantages and valuable results obtainable through my invention will hereinafter be referred to or will be apparent.

It may here be particularly mentioned that by the employment of my invention tungsten lamps of 16 candle power or less adapted for operation with an efficiency of about one watt per Hefner candle at such high voltages as 220 or more may be produced very readily, whereas heretofore it has been difficult or impossible to make such lamps, and even difficult to produce 16 candle power lamps having tungsten wire filaments for 110 volts and the like.

According to my invention, at least a part of the reduction in size by which tungsten wires or filaments of the desired fineness are finally obtained is effected chemically. It is not, however, necessary that the wires or filaments consist of chemically pure tungsten, but they may contain small quantities of foreign components,—for example, phosphorus or refractory oxides (lime, thorium). Indeed, these admixtures militate against the well-known crystalline structure characteristic of ordinary tungsten metal,—which interferes with the chemical treatment just referred to,—and so

are even useful in my process as a means of securing filaments or wire without this structure. In my process, the crystalline structure of ordinary tungsten metal is got rid of before the metal is subjected to chemical treatment,—which may be done by mechanical working of the metal while hot, as set forth in great detail in British Patent No. 23,499 of 1909.

The tungsten metal which has been deprived of its crystalline structure by mechanical working in a heated condition may be brought to a very small diameter by rolling or drawing and then subjected to the action of chemical means which (acting upon the surface) removes a considerable part of the mass of the wire or ribbon. The wire may thus be drawn to a diameter of about 5/100 to 3/100 millimeters and the reduction in size carried on chemically after that. Drawing to the diameter just mentioned is not fraught with any special difficulty, whereas drawing to still smaller sizes involves continually increasing difficulties and finally becomes impracticable because of the fact that the manufacture of the bored diamonds necessary for the very smallest diameters is no longer possible. Thus the second part of the process comes into use where the first part of the process becomes uneconomical or fails.

Chemical treatment of the wire may also be carried out in several stages with intervening drawing operations. This has the advantage of reducing the number of dies required and the amount of die wear, as well as various other advantages. Furthermore, the chemical treatment of the wire cannot well be continued uninterrupted so far that the wire is brought to a very small fraction of its initial cross-section, because then the original inequalities in the wire previous to the chemical reduction become more prominent, even without the production of inequalities by the chemical process itself. If, for example, the wire coming from the die is 100/1000 mm. thick at one end and 101/1000 mm. thick at the other (as may result from the enlargement of the die by wear during the drawing of the wire), then not only are the absolute differences preserved in the chemical or electro-chemical reducing process, but the differences become relatively greater when the wire is brought

2  
to a smaller diameter—for example, to 30/1000 mm. For whereas the inequality at first amounted to 1% of the diameter, at the end of the chemical reducing process it will 5 amount to about 3% of the diameter; and the difference in sectional area at the ends of the wire will have increased in even greater proportion. It is for these reasons that after having been brought to a certain 10 diameter by drawing the wire is advantageously reduced in size chemically, or electro-chemically, then drawn again to obviate or correct the relatively increased deviation in caliber, and then once more subjected to 15 the chemical reducing process. This alternation of the steps of the process may be carried out as often as desired until the desired fineness of the wire is attained. The drawing which takes place between each two 20 chemical or electro-chemical reducing operations may consist of a single drawing operation or of a plurality of such operations; and the process may in general be so conducted that the available diamond dies shall 25 be utilized to the best advantage. If, for example, a large number of dies with the diameter  $a$  have accumulated in the course of work and there is a deficiency of dies with a larger or smaller diameter  $b$ , then 30 the chemical or electro-chemical reduction will be carried so far that after it the dies may be used which are available in the greatest number. Thus not only is there a reduction 35 in the work of drawing, but also an economy of stones.

40 My invention will best be understood in connection with the accompanying drawing which illustrates one form of apparatus which may be used in carrying out my invention, and in which—

Figure 1 is a longitudinal section of the apparatus; and Fig. 2 is a transverse section along the line 2—2 of Fig. 1.

45 In the description (presently to be given) of how the chemical reduction in size may be effected, I have referred to the wire treated as so far reduced by the prior mechanical working that the chemical reduction may be carried out uninterrupted until the wire is 50 brought to the final size, according to the mode of employing my invention first above referred to. Before entering upon this description, I desire to call attention to certain facts, the knowledge of which may be generally serviceable in the carrying on of my 55 process.

60 It is necessary that the mechanical working result in the breaking up of the crystalline structure of the metal. If a tungsten wire of this sort which has been drawn down to about 5/100 millimeters or less is subjected to a glowing operation, it will generally change its structure again after a longer or shorter time and become crystalline,— 65 usually in a few seconds. In this changed

recrystallized condition, the second part of the process cannot be carried out with success; for although with suitable chemicals corrosion readily takes place, it does not go on uniformly, but scales out the crystals and attacks different places between the crystals with different intensity, and gives an uneven product of very irregular cross-section, with projecting crystal-points and edges, deep indentations and cracks,—in a word, 75 an unserviceable product. Again, if a tungsten wire is made, for example, by drawing a nickel-tungsten alloy into wire and expelling the nickel by heating in an inert gas or in vacuum, a uniform slender wire can 80 not be obtained therefrom by corrosion, since wire produced in this way is attacked very irregularly in consequence of its crystalline structure. It will, therefore, be seen that the absence of the crystalline structure is a 85 fundamental condition for the production of this very fine wire.

I may now proceed to indicate in some detail how the chemical reduction in size may be effected.

90 After the completion of the mechanical working in a glowing condition and the drawing to about 5/100 to 3/100 millimeters, the wire may for the further reduction in size be put (as a general thing) in a bath 95 containing an oxidizing means. As tungsten is an acid-forming element, of course an alkaline bath is particularly suitable; and although the corrosion can also be carried out with very powerful and oxidizing acids, 100 yet practically such an expedient will hardly be resorted to, for the corrosion in alkaline solutions is extremely convenient and certain. Very suitable, for example, is an alkaline solution of ferro-cyanid of potassium 105 (red prussiate of potash),—which is used in a state of considerable dilution in order to allow the corrosion to go on slowly, because then the time when the process should be stopped in order to obtain the desired diameter can be gaged much more easily than if concentrated solutions which act too rapidly are employed. Instead of the ferro-cyanid of potassium solution, the most 110 widely different alkaline oxidizing means may be used,—as, for example, persulfates, peroxids, etc. Potassium permanganate may also be used, especially if provision is made in a suitable manner for removing the coatings of manganese which precipitate on the 115 wire. It is very advantageous to pass the wire through an alkaline bath at a uniform rate. By the speed of passage the rapidity of the corrosion and consequently the diameter that will be obtained are determined. 120

125 It is not necessary to put oxidizing means in the bath; the chemical reduction in size may also be effected electrolytically. In this case the tungsten wire must, of course, form the anode. The wire is passed through the 130

bath at a slow, uniform rate and is properly to be taken over quite a large number of like poles (anodes) in such a manner that there is sufficient contact with them for current to be supplied at various points on the wire, since by reason of the very small diameter of the wire potential differences otherwise arise which may cause a lack of uniformity in the corrosion (though this tendency is checked by the uniform rate of passage through the bath). The wire may, for example, be alternately taken vertically into the bath and out again in a rising and descending (zigzag) line, and outside the vessel it may run over a number of contacts (anodes),—rollers for example,—which supply the positive current, so that uniform eating away of the relatively short loops which are in the liquid between each two rollers is insured. The loops are advantageously stretched in the bath over rollers, for example, which are non-conductors of electricity, or which consist of metal for which the voltage employed is not sufficient to enable current to pass into the liquid. The series or row of contacts by which current is supplied to the wire during its passage through the bath may be in parallel electrically. Tungsten wire without crystalline structure can also be reduced in gases, as chlorin for example, if the temperature is maintained sufficiently high to volatilize the chlorid formed.

To describe an example of how the chemical reduction treatment of the wire may be carried out electrolytically for sizes smaller than those above specifically referred to, 1-1/2 mil. drawn tungsten wire—that is, wire of a diameter of one and one-half one-thousandths of an inch—is passed through a dilute ammonia solution (20 parts concentrated ammonia to 80 parts water) at the rate of about 160 feet per hour. The apparatus illustrated in the drawing is suitable for carrying out this operation. The wire 10 is passed through an ammonia solution contained in a tin box 11 which serves as cathode for a current of 0.29 amperes and 2 volts of which the wire is anode. The wire is wound back and forth in ten loops over suitably separated cylinders 12 and 13 arranged one above the other on an insulating frame 14 of ebonite or similar material, about six to seven feet of wire being in the solution at once. The lower roll 12 is made of glass, and the upper roll 13 is made with longitudinal wires or bars 15 on the surface so that the points of contact between the roll and the filament are electrically in parallel, the contacting metal portions 15 being of platinum iridium. Current is led to the bars through a conducting core 16 and conducting bearing 17 to which the positive pole of the battery is connected. By a single passage of 1-1/2 mil. wire through the solu-

tion under these conditions it will be reduced to a size of about one mil. or one one-thousandth of an inch.

The tungsten wire which is the subject of my invention finds the most diverse applications. As its tensile strength and also its resistance to heat and to acids is very considerable, it may serve for suspension wires for fine measuring instruments (single and double-wire balances), torsion instruments of any kind, for reticles in optical instruments, and finally (as above referred to) for illuminating bodies for electric incandescent lamps and the like.

When the fine tungsten wire is to be used in incandescent lamps, it may after drawing to 5/100 to 3/100 mm. (for example) be placed upon the usual supporting means of the lamp,—which may have the form of the well known supporting frame used in tantalum lamps,—and then put in the bath containing chemicals adapted by their action to reduce the wire in size uniformly, so that a more slender wire of uniform surface and uniform cross-section throughout may result. On account of the material of the holders and the conducting wires, the reduction will in practice not be carried on in an acid solution, since only the strongest oxidizing acids (as concentrated nitric acid) act on the tungsten filament. Such a course is not necessary, however, since alkaline solutions are very well adapted to produce a uniform reduction. A dilute alkaline solution of red prussiate of potash (ferrocyanid of potassium) is very suitable, or an alkaline persulfate solution. The reduction proceeds gradually, and—particularly when a dilute reducing means is used—the process may be stopped at any desired moment, and lamps of any desired small current intensity may thus be produced from a given wire. It is easy to observe and follow the constantly changing electrical resistance of the filament. Thus the mounted filament may be dipped in a solution of potassium ferricyanid or potassium ferro-cyanid (about a 5-10% solution) until its cold resistance is doubled, which takes about five minutes.

The chemical reduction in size may also be performed in a bath which itself does not attack the tungsten if the tungsten wire is made the anode and a very weak current of a few milliamperes or even fractions thereof is conducted through the bath for a considerable time. Regard must be had for the fact that the resistance of the tungsten wire is so great that with stronger currents the current must be supplied at different points in order to avoid an irregular reduction.

Though in describing above how my invention can be carried out and applied I have referred to tungsten wire; tungsten ribbon can of course be produced in a similar

manner. Such ribbon has many uses more or less like those of tungsten wire.

What I claim as new and desire to secure by Letters Patent of the United States, is:—

- 5 1. The method of producing very fine tungsten wire of uniform surface and cross-section which consists in reducing the size of slender tungsten wire free from the ordinary crystalline structure of tungsten 10 by electrolytic corrosion.
2. The method of producing very fine refractory metal wire of uniform diameter and surface which consists in subjecting slender wire that has been deprived of its 15 crystalline structure by mechanical working to electrolysis, as anode in a bath of suitable electrolyte.
3. The method of producing very fine tungsten wire of uniform diameter and surface which consists in electrolytically corroding slender tungsten wire which has been deprived of its crystalline structure by mechanical working while hot by passing it at a uniform rate of speed through an alkaline 20 bath as anode in such a manner that a considerable length of wire is in the bath while supplying current to the wire at a number of points from a plurality of electrically 25 parallel anode contacts traversed by the

wire in its passage through the bath, so as to obtain a uniform corrosion.

4. The method of producing very fine tungsten wire of uniform diameter and surface which consists in reducing the size of tungsten wire, the metal of which has been deprived of its crystalline structure by mechanical working while hot by successive stages of electrolytic corrosion with suitable electrolyte, and counteracting the relative magnification of the inequalities of the wire resulting from this electrolytic reduction in size by drawing of the wire between the stages of the electrolytic treatment.

5. The process of producing very fine tungsten wire of uniform surface and cross-section which consists in repeatedly hot-working a body of tungsten to change its structure from crystalline to fibrous and at the same time to reduce its cross-section and then further reducing its cross-section by 45 electrolysis with said wire as anode.

In witness whereof, I have hereunto set my hand this 17th day of January, 1912.

DR. FRITZ BLAU.

Witnesses:

WOLDEMAR HAUPT,  
HENRY HASPER.